# EUROPEAN PATENT SPECIFICATION

(11) **EP 2 847 358 B1**
(45) Date of publication and mention of the grant of the patent: **04.03.2020**
(21) Application number: 13720957.3
(22) Date of filing: 07.05.2013
(51) Int. Cl.: C21D 6/00, C21D 1/20, C22C 38/26, C22C 38/28, C22C 38/38, C22C 38/44, C22C 38/46, C22C 38/48, C22C 38/50, C22C 38/54, C22C 38/58, C22C 38/02, C22C 38/22, C22C 38/24, C22C 38/04, C21D 1/00

(54) **TOUGH BAINITIC HEAT TREATMENTS ON STEELS FOR TOOLING**
SCHWERE BAINTWÄRMEBEHANDLUNGEN VON STÄHLEN ZUM PUNZEN
TRAITEMENTS THERMIQUES BAINITIQUES RÉSISTANTS SUR DES ACIERS POUR OUTILLAGE

(30) Priority: 07.05.2012 EP 12166949
(43) Date of publication of application: 18.03.2015
(73) Proprietor: Valls Besitz GmbH, 12205 Berlin (DE)
(72) Inventor: VALLS ANGLÉS, Isaac, 12205 Berlin (DE)
(74) Representative: Elzaburu S.L.P.
(86) International application number: PCT/EP2013/059542
(87) International publication number: WO 2013/167628

(56) References cited:
- EP-A1- 2 065 483
- EP-A1- 2 270 245
- GB-A- 999 866
- JP-A- 11 269 603
- JP-A- 2000 226 635
- JP-A- 2006 104 519
- JP-A- 2008 095 190

## Description

### Field of the invention

The present invention relates to the application of tough fully and partially bainitic heat treatments on certain steels, often alloyed tool steels or steels that can be used for tools and in particular hot work tool steels. This heat treatment strategy allows obtaining a fairly homogeneous distribution of properties through heavy sections. The resulting microstructures present high toughness. The present invention is also often applied to high toughness plastic injection moulding and structural steels and even to cold work and highspeed steels.

### Summary

Tool steels often require a combination of different properties which are considered opposed. A typical example can be the yield strength and toughness. For most tool steels the best compromise of such properties is believed to be obtainable when performing a purely martensitic heat treatment followed by the adequate tempering, to attain the desired hardness.

For heavy sections it is often impossible to attain pure martensitic microstructure through the whole cross-section, and very often it is not even possible to attain such a microstructure at the surface. In some tool steels, mixed microstructures with bainite and martensite have a particularly low fracture toughness which is very detrimental for several applications, like for example those where thermal fatigue is a dominant failure mechanism.

For most tool steels to attain a martensitic microstructure trough a heavy section implies the employment of very severe cooling that can easily lead to cracking.

In most applications, hardness (i.e mechanical resistance or yield strength) and toughness (resilience or fracture toughness) are not the only relevant material property for the tool steel, but some other properties are as relevant or at least relevant enough to be taken into account when designing the tooling solution. Such properties can be: resistance to working conditions (corrosion resistance, wear resistance, oxidation resistance at high temperatures,...), thermal properties (thermal diffusivity, thermal conductivity, specific heat, heat expansion coefficient,...), magnetic and/or electric properties, temperature resistance and many others. Often these properties are microstructure dependent and thus will be modified during heat treatment. So heat treatment is optimized to render the best property compromise for a given application.

Wear in material shaping processes is, primarily, abrasive and adhesive, although sometimes other wear mechanisms, like erosive and cavitative, are also present. To counteract abrasive wear hard particles are generally required in tool steels, these are normally ceramic particles like carbides, nitrides, borides or some combination of them. In this way, the volumetric fraction, hardness and morphology of the named hard particles will determine the material wear resistance for a given application. Also, the use hardness of the tool material is of great importance to determine the material durability under abrasive wear conditions. The hard particles morphology determines their adherence to the matrix and the size of the abrasive exogenous particle that can be counteracted without detaching itself from the tool material matrix. The best way to counteract the adhesive wear is to use FGM materials (functionally graded materials), normally in the form of ceramic coating on the tool material. In this case, it is very important to provide a good support for the coating which usually is quite brittle. To provide the coating with a good support, the tool material must be hard and have hard particles. In this way, for some industrial applications, it is desirable to have a tool material with high thermal diffusivity at a relatively high level of hardness and with hard particles in the form of secondary carbides, nitrides and/or borides and often also primary hard particles (in the case to have to counteract big abrasive particles).

In some applications the resistance to the working environment is more focused on corrosion or oxidation resistance than wear although both often co-exist. In such cases oxidation resistance at the working temperature or corrosion resistance against the aggressive agent are desirable. For such applications corrosion resistance tool steels are often employed, at different hardness levels and with different wear resistances depending on the application.

Thermal gradients are the cause of thermal shock and thermal fatigue. In many applications steady transmission states are not achieve due to low exposure times or limited amounts of energy from the source that causes a temperature gradient. The magnitude of thermal gradient for tool materials is also a function of their thermal conductivity (inverse proportionality applies to all cases with a sufficiently small Biot number).

Hence, in a specific application with a specific thermal flux density function, a material with a superior thermal conductivity is subject to a lower surface loading, since the resultant thermal gradient is lower. The same applies when the thermal expansion coefficient is lower and the Young's modulus is lower.

Traditionally, in many applications where thermal fatigue is the main failure mechanism, as in many casting or light alloy extrusions cases, it is desirable to maximize conductivity and toughness (usually fracture toughness and CVN).

Most forging applications use hardness in the 48-54 HRc range, plastic injection molding is preferably executed with tools having a hardness around 50-54 HRc, but for big plastic injection moulds often 30-45 HRc pre-hardened materials are used, die casting of zinc alloys is often performed with tools presenting a hardness in the 47-52 HRc range, while brass and aluminium are more often cast in dies with 35-49 HRc, hot stamping of coated sheet is mostly performed with tools presenting a hardness of 48-54 HRc and for uncoated sheets 54-58 HRc. For sheet drawing and cutting applications the most widely used hardness lies in the 56-66 HRc range. For some fine cutting applications even higher hardness are used in the 64-69 HRc. In almost all instances of the different applications described in this paragraph, either resilience, fracture toughness or both are of great significance.

One additional advantage of bainitic heat treatments is that they can be attained with a less abrupt quenching rate. Also for some tool steels they can deliver a similar microstructure trough a thicker section. For some tool steels with a retarded bainitic transformation it is possible to attain a perfectly homogeneous bainitic microstructure trough an extremely heavy section.

Unfortunately, it is well known that tool steels with microstructures presenting a considerable portion of bainite in the martensitic intended microstructure present low toughness and in particular low fracture toughness.

Nonetheless, bainite can be very fine and deliver high hardness and toughness if the transformation occurs at low enough temperatures. Many applications require high toughness, whether resilience or fracture toughness. In plastic injection applications often thin walls (in terms of resistant cross-section) are subjected to high pressures. When those walls are tall a big moment is generated on the base that often has a small radius, and thus high levels of fracture toughness are required. In hot working applications, the steels are often subjected to severe thermal cycling, leading to cracks on corners or heat checking on the surface. To avoid the fast propagation of such cracks it is also important for those steels to have as high as possible fracture toughness at the working temperature. Many efforts have been placed to attain purely martensitic structures in such applications, either through proper alloying to delay bainitic transformation kinetics, or through the development of methods to increase the cooling rate but avoiding cracking. The authors have observed that what is quite detrimental for toughness, and especially fracture toughness is the mixture of martensite and bainite, even for small quantities of the later. But if bainite is the only phase present, or at least strongly dominant, and especially if the bainite is a fine lower bainite then very high values of toughness can be attained, also fracture toughness at high temperatures. The authors have also observed that even for higher and coarser bainite, when the alloying level is high enough and the proper tempering strategy is followed, then most of the coarse cementite can be replaced by finer carbides and good toughness values achieved especially at higher temperatures. As mentioned martensitic heat treatments are often difficult to attain for heavy sections, or they might involve alloying which is detrimental for other properties.

The inventors have observed that a possible way for attaining uniform high toughness values in tooling requiring heavy sections and high mechanical properties is through the achievement of an at least 70% bainitic microstructure (preferably more than 80% and even more than 90%) on tool steels, or likely highly alloyed steels, with a low enough martensite start of transformation temperature and attaining most of the bainitic transformation at a temperature close enough to the martensite start of transformation temperature as to have a fine bainitic microstructure. Alternatively for applications requiring the toughness at higher temperatures, the problem can be solved with the presence of enough alloying elements and the proper tempering strategy to replace most Fe3C with other carbides and thus attaining high toughness even for coarser bainite. Also the traditional way can be used in certain instances, consisting in avoiding coarse Fe3C and/or its precipitation on grain boundaries with the additions of elements that promote its nucleation like Al, Si.... It is also advantageous for most applications to use thermo-mechanical treatments leading to the refining of the final grain size.

### State of the art

Super-bainitic or high strength bainitic steels are low alloy steels developed by H.K.D.H. Bhadeshia et al. where low temperature bainitic transformations are used to attain high mechanical properties (as an example can be taken: Very strong low temperature bainite, F.G. Caballero, H.K.D.H. Bhadeshia et al., in: Materials Science and Technology, March 2002, Vol. 18, Pg. 279-284 . DOI 10.1179/026708301225000725). They are steels with low martensite transformation start temperature mostly due to their high carbon contents, and with slow transformation kinetics for equilibrium phases (especially ferrite/perlite and upper bainite). The tool steels of the present invention rely on higher alloying for the attaining of the desirable mechanical properties, and normally lower %Ceq contents. As a consequence the transformation temperatures for the present invention are often higher leading to lower mechanical strength in the "as quenched" condition, which is not normally the condition of usage.
JP2000226635 A discloses a hot tool steel with a high level of temperature strength and toughness. The structure at the time of quenching is formed of martensite + bainite, with a bainitic rate of 5 to 80%.

### Detailed description of the invention

The present invention is based on a combination of alloying and heat treatments and how those heat treatments are applied. The preferred microstructure is predominantly bainitic, more than 80%, more preferably 86% vol% and even more preferably more than 92% vol%, since is normally the type of microstructure easier to attain in heavy sections and also because it can be very tough when following the indicated steps.
For some applications, especially those requiring heavy sections with materials presenting limited hardenability in the bainitic regime, High Temperature bainite will be preferred since it is the first bainite to form when cooling the steel after austenitization. In this document High Temperature bainite refers to any microstructure formed at temperatures above the temperature corresponding to the bainite nose in the TTT diagram but below the temperature where the ferritic/perlitic transformation ends. Although in literature High temperature bainite just refers to upper bainite, in the present invention both upper and lower bainite are referred, the last one which can occasionally form in small amounts also in isothermal treatments at temperatures above the one of the bainitic nose. For the applications requiring high easy hardenability, the high temperature bainite should be the majoritary type of bainite and thus from all bainite is preferred at least 50% vol%, preferably 65% vol%, more preferably 75% vol% and even more preferably more than 85% vol% to be High Temperature Bainite. As it is well known in metallurgical terms, bainite is one of the decomposition products when austenite is not cooled under thermodinamical equilibrium. It consists on a fine non-lamellar structure of cementite and dislocation-rich ferrite plates as it is a non-diffusion process. The high concentration of dislocations in the ferrite present in the bainite makes this ferrite harder than it would normally be. Often high temperature bainite will be predominantly. Upper bainite refers to the coarser bainite microstructure formed at the higher temperatures range within the bainite region, to be seen in the TTT temperature-time-transformation diagram, which in its turn, depends on steels composition. Fine bainite refers qualitatively to the size of the plates or laths of ferrite, which in this case mean small; On the contrary, for big lath sizes bainite is known as coarse bainite. On the other hand, stable phases like ferrite or perlite are in general terms not very desirable structures to achieve during heat treating. The inventors have seen that a way to increase the toughness of the High Temperature Bainite, including the Upper and lower Bainite is to reduce the grain size, and thus for the present invention when tough upper bainite is required grain sizes of ASTM 8 or more, preferably 10 or more and more preferably 13 or more are advantageous. The inventors have also seen that surprisingly high values of toughness can be attained with High Temperature Bainite when using microstructures where cementite has been suppressed, strongly reduced and/or its morphology altered to finer lamella or even more so when the cementite is globulized. For bainites including retained austenite, the same applies for the morphology of the retained austenite phase. This is what is referred as Tough High Temperature Bainite in this application: small grain size high temperature bainite and/or low cementite bainite and/or fine lamella or globular morphology high temperature bainite. For some applications it is clearly preferred to have most of the high temperature bainite being tough high temperature bainite more than a 60%, preferably more than a 78%, and even more preferably more than a 88% in volume percent. The inventors have seen that specially for low %Si alloys (lower than 1%, specially lower than 0,6% and even more specially lower than 0,18%), high contents of globular bainite provide very high resilience which is of high interest for several applications, in this case it is desirable to have 34% of all bainite or more to be of globular morphology, preferably 55% or more, more preferably 72% or more and more preferably 88% or more. In some instances it is even possible to have all bainite having a globular morphology. When combined with small grain size as described above for the High Temperature Bainite in general, even unexpected high values of fracture toughness can be attained. For some applications having some ferrite and or perlite is not too detrimental, but for most applications no ferrite/perlite will be desirable or at the most 2% or eventually 5%. The applications more tolerant to ferrite/perlite can allow up to 10% or even 18%. In a bainitic microstructure generally the presence of martensite leads to a decrease in fracture toughness, for applications where fracture toughness is not so important there is no restrictions on the fraction of bainite and martensite, but the applications where fracture toughness matters on predominantly bainitic microstructures will prefer the absence of martensite or at most its presence up to 2% or eventually 4%. For some compositions 8% or even 17% of martensite might be tolerable and yet maintaining a high fracture toughness level. If high fracture toughness at lower temperatures is desirable, in heavy cross sections, there are two possible strategies to be followed for the steels of the present invention within the predominantly bainitic heat treatments. Either alloy the steel to assure the martensitic transformation temperature is low enough (normally lower than 480°C, preferably lower than 400°C, more preferably lower than 340°C, further more preferably lower than 290°C and even lower than 240°C. For extremely fine bainite, but often associated to very slow transformation kinetics the transformation temperature should be below 220°C, preferably below 180°C and even below 140°C), and all transformation kinetics to stable not so desirable structures (ferrite/perlite, upper bainite) slowly enough (at least 600 seconds for 10% ferrite/perlite transformation, preferably more than 1200 seconds for 10% ferrite/perlite transformation, more preferably more than 2200 seconds for 10% ferrite/perlite transformation and even more than 7000 seconds for 10% ferrite/perlite transformation. Also more than 400 seconds for 20% transformation into bainite, preferably more than 800 seconds for 20% bainite, more preferably more than 2100 seconds for 20% bainite and even more than 6200 seconds for 20% bainite) to be able to make a predominantly fine bainite (at least 50% vol%, preferably 55% vol%, more preferably 60% vol% and even more preferably more than 70% vol%) heat treatment. Alternatively the alloying content regarding elements with higher propensity than Fe to alloy with %C, %N and %B has to be chosen to be high enough. Elements having an affinity for carbon higher than iron are Hf, Ti, Zr, Nb, V, W, Cr, Mo as most important ones and will be referred in this document as strong carbide formers (special attention has to be played since this definition does not coincide with the most common one in the literature where often Cr, W and even Mo and V are often not referred as strong carbide formers). Elements with higher carbon affinity than Fe will form their respective carbides or a combination of them before the iron carbide can form, from now on referred to as alloyed carbides. Depending on the carbide itself, properties can vary. Special cases are later on and depending on the particular properties sought, properly described. In this sense, most significant are the presence of %Moeq, %V, %Nb, %Zr, %Ta, %Hf, to a lesser extend %Cr and all other carbide formers. Often more than a 3% in the sum of elements with higher affinity for carbon than iron will be present, preferably more than a 6.2%, more preferably more than 7.2% and even more than 8.4%. Additionally any thermo-mechanical treatment leading to a refining of the final grain size is advantageous, especially for predominantly bainitic heat treatments because then the effect is not only in the improvement of toughness but also in the increase of hardenability, the same can be said for treatments avoiding carbide precipitation on grain boundaries. Such a treatment can be, for example, a first step at high temperatures above 1.020 °C to coarsen the austenite grain size (since it is a diffusion process the higher the temperature the lower the time required, strain can also be introduced trough mechanical deformation but recrystallization avoided at this point). Then the steel is cooled fast enough to avoid transformation into stable microstructures (ferrite/perlite, and also bainite as much as possible) and also to minimize carbide precipitation. Finally the steel is stress released at a temperature close to Ac1. This will promote the nucleation of very fine grains in the final heat treatment, especially if it is predominantly bainitic.

There are quite some reports in the literature about the existence of very tough lower bainite under some quite restrictive conditions that lead to poor tribological performance for some applications. The inventors have seen that this can be solved with the usage of alloyed carbides, when %C is well equilibrated as explained in more detail later. In general for those applications it is desirable to have a 3% or more carbide formers stronger than iron, preferably a 3,2% or more, more preferably a 4,6 or more or even a 7,6 or more. There are even fewer reports in the literature of the existence of tough bainite structures in the high temperatue bainite regime, like for example globular or globalized bainite, and it is always associated to low %C contents, normally in the range of %C < 0,2 in weight percent. While this structure is very desirable for many applications in the present invention, most of those same applications require mechanical and tribological properties which are with extreme difficulty attained with such low %C contents. The inventors have seen that surprisingly in the current invention such structures can be attained for considerably higher %C contents. It is a peculiarity of the present invention to have simultaneously tough high temperature bainite and more than 0,21% weight %C, preferably more than 0,26%, more preferably more than 0,31%, even more preferably more than 0,34%, and even more than 0,38%. The way this is achieved is by having some of the nominal %C -The theoretical total %C of the steel - not participate the austenite to bainite transformation, One effective way to do so is to have some of the %C bound to carbides right before the transformation starts and during the transformation. This can be accomplished by not dissolving all carbides during the austenization, or by performing a controlled cooling so that carbide precipitation takes place before the bainitic transformation. In this sense, it is advantageous for some applications of the present invention to have 5% or more of the nominal weight %C in the form of carbides formed before the bainitic transformation, preferably 8% or more, more preferably 12% or more and even 23% or more. Note that in metallurgical terms, composition of steels is normally given in terms of Ceq, which is defined as carbon upon the structure considering not only carbon itself, or nominal carbon, but also all elements which have a similar effect on the cubic structures of the steel, normally being B, N. During last description, carbon was meant to be just carbon content, or nominal carbon.

Martensitic or bainitic microstructures are often rather brittle right after quenching and one way to recover some ductility and/or toughness is by tempering them. In this text references are made to tempered martensite and tempered bainite, with this terminology in this text is referred a martensite and/or bainite that has undergone any type of heating after forming (during the quenching process). This heating leads at first to a relaxation of the structure, followed by a migration of the carbon atoms (often the resulting microstructures are given particular names in the literature: Troostite, Sorbite....), transformation of the retained austenite if present, precipitation of alloyed carbides and/or morphology change and redisolution of any type of carbides (cementite and alloyed carbides included) amongst others. Which mechanisms actually take place and to what extend depends on the steel composition, original microstructure and the temperature and time of the tempering cycles applied. So any heating after quenching (formation of the bainite) leads to the in this text called tempered tempered Bainite. Often during the implementation of the present invention a tempering (which might be a multiple one) takes place during the manufacturing of the steel, and another tempering (which again might be a multiple one) takes place during the usage of the steel to manufacture a component or tool.
The austenitization temperature for tool steels is normally well above Ac3 since it is often convenient to bring most carbides into dissolution before quenching. Depending on final application, it will be more interesting to austenitise at lower temperatures, even between AC1 and AC3 (where an incomplete austenitization takes place). Typically the austenitization temperatures will be above AC3, but often below the temperature of complete carbide dissolution, even in absence of primary carbides, as grain growth is directly proportional to temperature. Small grains sizes are normally accompanied by higher strength so lower temperatures are more convenient for this purpose. If it is accompanied with short time, once the core has reached the temperature, even better. For some applications, these values are below 1040 °C, preferably below 1020 °C and even below 990 °C. On the contrary and depending on steel's composition, if austenitization temperature is smaller than the dissolution temperature of some kind of carbides, for example M₆C carbides, carbides do not have the possibility of redistributing themselves along the matrix. High temperature carbides tend to agglomerate caused by metallurgical segregations and it normally has a negative effect on toughness. Better performance of carbides is found for small sizes, due to an increase of strength through phase boundaries. It is even better if embodiment within the matrix is homogeneous all along. Therefore, for some applications it is more convenient to ensure a maximum dissolution of carbides into austenite so that the precipitate at the desired place during the next steps of the heat treatment. Typical values are above 1080 °C, for some composition of this invention above 1110 °C and even above 1120 °C. The heating up and austenitization can be carried out in any type of furnace, atmospheric, protected atmosphere, salt bath, vacuum..... Uneven heating or overheating from specified temperature should be avoided. Heating rate must be controlled, specially around the AC3 range because contraction of the body centered cubic structure from ferrite transforms to the face centered cubic structure of austenite may produce micro cracks that can grow afterwards.

Once the austenization has been performed in the preferred way, the material is subjected to a rapid cooling to an intermediate temperature or transformation temperature Tᵢₙₜ. This cooling has to be fast enough so that no massive ferrite transformation occurs during the process. For this purpose, it is possible to change the piece to another furnace running at the specified temperature, cool by means of a salt bath among any others which guarantees that no stable phases like ferrite and/or pearlite take place. Normally less than 20% ferrite or stable phases is desirable, more preferably less than 12% and most preferred is less than 2% or even none. The holding at this temperature has to be long enough to minimize the transformation of austenite to martensite. At least 1.5h or more, preferably 10h or more, more preferably 24h or more and even more preferably 72h or more. Sometimes, depending on the size of the pieces, as well as its final application, even larger holding times are recommended, preferably 90h, more preferably 120h and even 200h. Tᵢₙₜ has to be in a range where lite or no martensite is able to form and most of final microstructure consists on bainitic microstructure with fine carbide-like constituients. Therefore, Tint has to be below the martensite start of transformation (Ms) + 300°C and above Ms - 50°C. Desired final structure has to be at lest 70% vol% bainitic microstructure, preferably 75% vol%, more preferably 86% vol% and even more preferably more than 92% vol%. It is very advantageous when the bainitic transformation is done at a temperature Tint below 400°C, attaining a final hardness above 45HRc.
Other preferred embodiments consist on a two step cooling from austenitizing temperature to room temperature, within the specified temperature range including. For this purpose and for this preferred embodiments, Tᵢₙₜ will be renamed as Tᵢₙₜ₁ and Tᵢₙₜ₂. Concerning upper limit for Tᵢₙₜ₁ it is desirable to be below 750°, more preferably below 620°C, more preferably below 590°C and even more preferably below 560°C, lower limit is desirable to be above 460°C, preferably above 495°C, more preferably above 512°C and even more preferably 523°C. The holding time at this temperature range (Tᵢₙₜ₁- Tᵢₙₜ₂) can vitiate from several minutes to several hours depending on the heat treated piece size and the lack of transformation at Tᵢₙₜ₁, desirably at least half an hour, preferably at least 1h, more preferably at least 2h and in some cases even more than 5h. In fact the only reason not to stay more time is an economical reason, it can stay several days at the selected temperature if desired Tᵢₙₜ₂ upper limit is desirably below 450°C, preferably below 420°C, more preferably below 320°C and even more preferably below 360°C. The lower limit is desirable to be below 350°C, preferably below 320°C, more preferably below 250 and even more preferably below 200°C.
Therefore, the present invention is a method to manufacture a steel, casting die or tool, comprising providing a steel with both a bainite and a martensite domain of existence, characterized in that the steel is subjected to a thermal treatment comprising the following steps:
a) Austenitization
b) Cooling rapid enough to avoid the formation of more than a 20% stable phases with a transformation temperature higher than bainite
c) Maintaining the temperature to transform at least 60% vol of remaining austenite between Ms+300°C and Ms-50°C, wherein Ms is the martensite start of transformation temperature;
wherein more than 80% of the microstructure is bainitic with fine carbide-like constituents with a CVN higher than 8 Joule within at least 20mm from the surface of the thermally treated steel, in line with attached claim 1.

The present invention is well suited for steels which have a martensite start (Ms) of transformation equal or lower than 540°C, preferably lower than 480°C, more preferably lower than 440 and even more preferably lower than 360°C.

The present invention is advantageous when thermal treatment is followed by at least one tempering cycle desirably above 500°C, preferably above 550°C, more preferably above 600°C and even more preferably above 620°C. Often more than one cycle is desirable. more preferably more than one cycle to separate the alloy cementite to dissolve the cementite in solid solution and to separate the carbide formers stronger than iron.

Alternatively for applications requiring the toughness at higher temperatures, the problem can be solved with the presence of enough alloying elements and the proper tempering strategy to replace most Fe3C with other carbides and thus attaining high toughness even for coarser bainite. Upon formation of the bainite the steel is tempered with at least one tempering cycle at a temperature above 500°C to ensure that a significant portion of the cementite is replaced by carbide-like structures containing carbide formers stronger than iron. Also the traditional way can be used in certain instances, consisting in avoiding coarse Fe3C and/or its precipitation on grain boundaries with the additions of elements that promote its nucleation like Al, Si....

In yet a further embodiment of the method of the invention, at least 70% of the bainitic transformation is made at temperatures below 400°C and/or the thermal treatment includes at least one tempering cycle at a temperature above 500°C to ensure separation of stronger carbide formers carbides, so that most of the attained microstructure, with the exception of the eventual presence of primary carbides, is characterized by the minimization of rough secondary carbides, in particular at least 60% in volume of the secondary carbides has a size of 250 nm or less, such that a toughness of 10 J CVN or more is attained.

In an additional embodiment of the method of the invention, the composition and tempering strategy is chosen so that high temperature separation secondary carbide types such as types MC, MC-like type as M4C3, M6C and M2C are formed, in such a manner that a hardness above 47 HRc is obtainable even after holding the material for 2h at a temperature of 600 °C or more.

In another additional embodiment of the method of the invention, the steel has a composition within the following range:
% Cr < 3.0
% Si < 0.8
wherein
%Mo + ½ · %W > 2.0.
and the tempering strategy is chosen to minimize carriers scattering, such that a low scattering structure characterized by a diffusivity of 8 mm²/s or more is obtainable even for a hardness of 45 HRc or more.

In yet another additional embodiment of the method of the invention, the steel has the following composition:
% Ni > 0.8

The steel produced according to the method of the invention presents at least two of the following features:
- it contains retained austenite;
- its cementite is not wholly dissolved in the solid solution;
- its cementite has not fully coalesced; and
- carbide formers stronger than iron are present in the solid solution,
so that the hardness of the steel can be raised in an amount of at least 4 HRc upon application of a later thermal treatment below austenitizing temperature.

The present invention is especially well suited to obtain steels for the hot stamping tooling applications. The steels of the present invention perform especially well when used for plastic injection tooling. They are also well fitted as tooling for die casting applications. Another field of interest for the steels of the present document is the drawing and cutting of sheets or other abrasive components. Also forging applications are very interesting for the steels of the present invention, especially for closed die forging. Also for medical, alimentary and pharmaceutical tooling applications the steels of the present invention are of especial interest.
The present invention suits especially well when using steels presenting high thermal conductivity (thermal conductivity above 35 W/mK, preferably 42 W/mK, more preferably 48 W/mK and even 52 W/mK), since their heat treatment is often complicated especially for large or complex in geometry dies. In such cases the usage of the present invention can lead to very significant costs savings, due to the levels of toughness not attainable in any other way, at least at high hardness levels and for heavy sections. The present invention is well indicated in particular when using high thermal conductivity steels, with the following composition all percentages being indicated in weight percent:

| | | | | | | | |
|---|---|---|---|---|---|---|---|
| %C_{eq} | = 0.16 - 1.9 | %C | = 0.16 - 1.9 | %N | = 0 - 1.0 | %B | = 0 - 0.6 |
| %Cr | < 3.0 | %Ni | = 0 - 6 | %Si | = 0 - 1.4 | %Mn | = 0 - 3 |
| %Al | = 0 - 2.5 | %Mo | = 0 - 10 | %W | = 0 - 10 | %Ti | = 0 - 2 |
| %Ta | = 0 - 3 | %Zr | = 0 - 3 | %Hf | = 0 - 3 | %V | =0 - 4 |
| %Nb | = 0 - 1.5 | %Cu | = 0 - 2 | %Co | = 0 - 6, | | |

the rest consisting of iron and trace elements wherein, $% {C}_{eq} = % ⁢ C + 0.86 ∗ % ⁢ N + 1.2 ∗ % ⁢ B ,$ characterized in that
%Mo + ½ · %W > 2.0.

In the meaning of the present specification, trace elements refer to any element, otherwise indicated, in a quantity less than 2%. For some applications, trace elements are preferable to be less than 1,4%, more preferable less than 0,9% and sometimes even more preferable to be less than 0,4%. Possible elements considered to be trace elements are H, He, Xe, Be, O, F, Ne, Na, Mg, P, S, Cl, Ar, K, Ca, Sc, Fe, Zn, Ga, Ge, As, Se, Br, Kr, Rb, Sr, Y, Tc, Ru, Rh, Pd, Ag, Cd, In, Sn, Sb, Te, I, Xe, Cs, Ba, La, Ce, Pr, Nd, Pm, Sm, Eu, Gd, Tb, Dy, Ho, Er, Tm, Yb, Lu, Re, Os, Ir, Pt, Au, Hg, Tl, Pb, Bi, Po, At, Rn, Fr, Ra, Ac, Th, Pa, U, Np, Pu, Am, Cm, Bk, Cf, Es, Fm, Md, No, Lr, Rf, Db, Sg, Bh, Hs, Mt alone and/or in combination. For some applications, some trace elements or even trace elements in general can be quite detrimental for a particular relevant property (like it can be the case sometimes for thermal conductivity and toughness), for such applications it will be desirable to keep trace elements below a 0,4 %, preferably below a 0,2%, more preferably below 0,14 % or even below 0,06%.

Some smaller ranges within the above mentioned compositional range are of special significance for certain applications. For example when it comes to the %Ceq content it is preferably to have a minimum value of 0.22% or even 0.33%. On the other hand for very high conductivity applications it is better to keep %C below 1.5% and preferably below 0.9%. %Ceq has a strong effect in reducing the temperature at which martensitic transformation starts, thus higher values of %Ceq will be desirable for either high wear resistance applications or applications where a fine bainite is desirable. In such cases it is desirable to have a minimum of 0.4% of Ceq often more than 0.5% and even more than 0.8%. If some other elements that reduce the martensite transformation temperature are present (like for example %Ni) then the same effect can be obtained with lower %Ceq (same levels as described before). Also the %Moeq (%Mo + ½ · %W) levels should be higher for maximum thermal conductivity, normally above 3.0% often above 3.5%, preferably above 4% or even 4.5%. But high levels of %Moeq do tend to shorten the bainitic transformation time. Also if thermal conductivity needs to be maximized is better to do so within a compositional range with lower %Cr, normally less than 2.8% preferably less than 1.8% and even less than 0.3%. A special attention has to be placed in elements that increase hardenability by slowing the kinetics of the austenite decomposition into ferrite/perlite. Very effective in this sense is %Ni and somewhat less %Mn. Thus for heavy sections it is often desirable to have a minimum %Ni content normally 1%, preferably 1.5% and even 3%. If %Mn is chosen for this goal higher amounts are required to attain the same effect. About double as much quantity is required as is the case for %Ni. For applications where the steel is to attain temperatures in excess of 400 °C during service it might be very interesting to have %Co present which tends to increase tempering resistance amongst others and presents the odd effect of affecting the thermal diffusivity positively for high temperatures. Although for some compositions an amount of 0.8% might suffice, normally it is desirable to have a minimum of 1,0% preferably 1,5% and for some applications even 2.7%. Also for applications where wear resistance is important it is advantageous to use strong carbide formers, then %Zr+%Hf+%Nb+%Ta should be above 0.2%, preferably 0.8% and even 1.2%. Also %V is good carbide former that tends to form quite fine colonies but has a higher incidence on thermal conductivity than some of the former, but in applications where thermal conductivity should be high but is not required to be extremely high and wear resistance and toughness are both important, it will generally be used with a content above 0.1%, preferably 0.3% and even more than 0.55%. For very high wear resistance applications it can be used with a content higher than 1.2% or even 2.2%.

So, for such kind of steels, unusually high final tempering temperatures end up being used, often above 600°C, even when hardness over 50 HRc are chosen. In steels of the present invention it is usual to achieve hardness of 47 HRc, even more than 52 HRc, and often more than 53 HRc and with the embodiments regarded as particularly advantageous due to their wear resistance, hardness above 54HRc, and often more than 56 HRc are possible with even one tempering cycle above 540°C, giving a low scattering structure characterized by a thermal diffusivity greater than 8 mm²/s and, generally, more than 9 mm²/s, or even more than 10 mm²/s, when particularly well executed then greater than 11 mm²/s, even greater than 12 mm²/s an occasionally above 12,5 mm²/s. As well as achieving hardness greater than 46 HRc, even more than 50 HRc with the last tempering cycle above 600°C, often above 640°C, and sometimes even above 660 °C, presenting a low scattering structure characterized by a thermal diffusivity higher than 10 mm²/s, or even than 12 mm²/s, when particularly well executed then greater than 14 mm²/s, even greater than 15 mm²/s and occasionally above 16 mm²/s. Those alloys can present even higher hardness with lowering tempering temperatures, but for most of the intended applications a high tempering resistance is very desirable. Actually the bainitic microstructure presents a markedly higher tempering resistance in this kind of steels. As can be seen in the examples with some very particular embodiments with high carbon and high alloying, leading to a high volume fraction of hard particles, hardness above 60 HRc with low scattering structures characterized by thermal diffusivity above 8mm²/s and generally more than 9mm²/s are possible in the present invention.

The present invention is also especially good indicated when using steels with the following composition range, all percentages being indicated in weight percent:

| | | | | | | | |
|---|---|---|---|---|---|---|---|
| %C_{eq} | = 0.15-3.0 | %C | = 0.15 - 3.0 | %N | = 0 - 1.6 | %B | = 0 - 2.0 |
| %Cr | > 4.0 | %Ni | = 0 - 6.0 | %Si | = 0 - 2.0 | %Mn | = 0 - 3 |
| %Al | = 0 - 2.5 | %Mo | = 0 - 15 | %W | = 0 - 15 | %Ti | = 0 - 2 |
| %Ta | = 0 - 3 | %Zr | = 0 - 3 | %Hf | = 0 - 3 | %V | = 0 - 12 |
| %Nb | = 0 - 3 | %Cu | = 0 - 2 | %Co | = 0 - 6, | | |

the rest consisting of iron and trace elements wherein, $% {C}_{eq} = % ⁢ C + 0.86 ∗ % ⁢ N + 1.2 ∗ % ⁢ B ,$

Some smaller ranges within the above mentioned compositional range are of special significance for certain applications. For example when it comes to the %Ceq content it is preferably to have a minimum value of 0.22%, preferably 0.28% more preferably 0.34% and when wear resistance is important preferably 0.42% and even more preferably 0.56%. Very high levels of %Ceq are interesting due to the low temperature at which martensite transformation starts, such applications favor %Ceq maximum levels of 1.2%, preferably 1.8% and even 2.8%. Applications where toughness is very important favor lower %Ceq contents, and thus maximum levels should remain under 0.9% preferably 0.7% and for very high toughness under 0.57%. Although a noticeable ambient resistance can be attained with 4% Cr, usually higher levels of %Cr are recommendable, normally more than 8% or even more than 10%. For some special attacks like those of chlorides it is highly recommendable to have %Mo present in the steel, normally more than 2% and even more than 3.4% offer a significant effect in this sense. Also for applications where wear resistance is important it is advantageous to use strong carbide formers, then %Zr+%Hf+%Nb+%Ta should be above 0.2%, preferably 0.8% and even 1.2%. Also %V is good carbide former that tends to form quite fine colonies but has a higher incidence on thermal conductivity than some of the former, but in applications where thermal conductivity should be high but is not required to be extremely high and wear resistance and toughness are both important, it will generally be used with a content above 0.1%, preferably 0.54% and even more than 1.15%. For very high wear resistance applications it can be used with content higher than 6.2% or even 8.2%.

The steels described above can be particularly interesting for applications requiring a steel with improved ambient resistance, especially when high levels of mechanical characteristics are desirable and the cost associated to heat treatment (both in terms of time and money) for its execution or associated distortions, are significant.
The present invention is also especially good indicated when using steels with the following composition range, all percentages being indicated in weight percent:

| | | | | | | | |
|---|---|---|---|---|---|---|---|
| %C_{eq} | = 0.15 - 2.0 | %C | = 0.15 - 0.9 | %N | = 0 - 0.6 | %B | =0 - 0.6 |
| %Cr | > 11.0 | %Ni | = 0 - 12 | %Si | = 0 - 2.4 | %Mn | = 0 - 3 |
| %Al | = 0 - 2.5 | %Mo | =0 - 10 | %W | =0 - 10 | %Ti | = 0 - 2 |
| %Ta | = 0 - 3 | %Zr | = 0 - 3 | %Hf | = 0 - 3 | %V | = 0 - 12 |
| %Nb | = 0 - 3 | %Cu | = 0 - 2 | %Co | = 0 - 12, | | |

the rest consisting of iron and trace elements, wherein %C_{eq} = %C + 0.86 ^{∗} %N + 1.2 ^{∗} %B,

Some smaller ranges within the above mentioned compositional range are of special significance for certain applications. For example when it comes to the %Ceq content it is preferably to have a minimum value of 0.22%, preferably 0.38% more preferably 0.54% and when wear resistance is important preferably 0.82%, more preferably 1.06% and even more than 1.44%. Very high levels of %Ceq are interesting due to the low temperature at which martensite transformation starts, such applications favor %Ceq maximum levels of 0.8%, preferably 1.4% and even 1.8%. Applications where toughness is very important favor lower %Ceq contents, and thus maximum levels should remain under 0.9% preferably 0.7% and for very high toughness under 0.57%. Although corrosion resistance for martensitic microstructure can be attained with 11% Cr, usually higher levels of %Cr are recommendable, normally more than 12% or even more than 16%. For some special attacks like those of chlorides and to enhance hardness gradient at the secondary hardness peak it is highly recommendable to have %Moeq present in the steel, often more than 0.4%, preferably more than 1.2% and even more than 2.2% offer a significant effect in this sense. Also for applications where wear resistance or thermal conductivity are important it is advantageous to use strong carbide formers, then %Zr+%Hf+%Nb+%Ta should be above 0.1%, preferably 0.3% and even 1.2%. Also %V is good carbide former that tends to form quite fine colonies but has a higher incidence on thermal conductivity than some of the former, but in applications where thermal conductivity should be high but is not required to be extremely high and wear resistance and toughness are both important, it will generally be used with a content above 0.1%, preferably 0.24% and even more than 1.15%. For very high wear resistance applications it can be used with content higher than 4.2% or even 8.2%.
The steels described above can be particularly interesting for applications requiring a steel with corrosion or oxidation resistance, especially when high levels of mechanical characteristics are desirable and the cost associated to heat treatment (both in terms of time and money) for its execution or associated distortions, are significant
The present invention is then especially good indicated when using steels with the following composition range, all percentages being indicated in weight percent:

| | | | | | | | |
|---|---|---|---|---|---|---|---|
| %C_{eq} | = 0.5 - 3.0 | %C | = 0.5 - 3.0 | %N | = 0 - 2.2 | %B | = 0 - 2.0 |
| %Cr | = 0.0 - 14 | %Ni | = 0 - 6.0 | %Si | = 0 - 2.0 | %Mn | = 0 - 3 |
| %Al | = 0 - 2.5 | %Mo | = 0 - 15 | %W | = 0 - 15 | %Ti | = 0 - 4 |
| %Ta | = 0 - 4 | %Zr | = 0 - 12 | %Hf | = 0 - 4 | %V | = 0 - 12 |
| %Nb | = 0 - 4 | %Cu | = 0 - 2 | %Co | = 0 - 6, | | |

the rest consisting of iron and trace elements wherein, $% {C}_{eq} = % ⁢ C + 0.86 ∗ % ⁢ N + 1.2 ∗ % ⁢ B ,$

Some smaller ranges within the above mentioned compositional range are of special significance for certain applications. For example when it comes to the %Ceq content it is preferably to have a minimum value of 0.62%, preferably 0.83% more preferably 1.04% and when extreme wear resistance is important preferably 1.22%, more preferably 1.46% and even more than 1.64%. Very high levels of %Ceq are interesting due to the low temperature at which martensite transformation starts, such applications favor %Ceq maximum levels of 1.8%, preferably 2.4% and even 2.8%. %Cr has two ranges of particular interest: 3.2%-5.5% and 5.7%-9.4%. To enhance hardness gradient at the secondary hardness peak it is highly recommendable to have %Moeq present in the steel, often more than 2.4%, preferably more than 4.2% and even more than 10.2% offer a significant effect in this sense. Also for applications where wear resistance or thermal conductivity are important it is advantageous to use strong carbide formers, then %Zr+%Hf+%Nb+%Ta should be above 0.1%, preferably 1.3% and even 3.2%. Also %V is good carbide former that tends to form quite fine colonies of very hard carbides, thus when wear resistance and toughness are both important, it will generally be used with a content above 1.2%, preferably 2.24% and even more than 3.15%. For very high wear resistance applications it can be used with content higher than 6.2% or even 10.2%.
The steels described above can be particularly interesting for applications requiring a steel with very high wear resistance, especially when high levels of hardness are desirable and the cost associated to heat treatment (both in terms of time and money) for its execution or associated distortions, are significant.
The present invention can be applied to low cost steels with the following composition, all percentages being indicated in weight percent:

| | | | | | | | |
|---|---|---|---|---|---|---|---|
| %C_{eq} | = 0.2 - 0.9 | % C | = 0.2 - 0.9 | %N | = 0 - 0.6 | %B | = 0 - 0.6 |
| %Cr | = 0.0 - 4.0 | %Ni | = 0 - 6.0 | %Si | = 0.2 - 2.8 | %Mn | = 0.2 - 3 |
| %Al | =0-2.5 | %Mo | =0 - 6 | %W | =0-8 | %Ti | =0-2 |
| %Ta | =0-2 | %Zr | =0-2 | %Hf | =0-2 | %V | =0-4 |
| %Nb | = 0 - 2 | %Cu | = 0 - 2 | %Co | = 0 - 6, | | |

the rest consisting of iron and trace elements wherein, $% {C}_{eq} = % ⁢ C + 0.86 ∗ % ⁢ N + 1.2 ∗ % ⁢ B ,$ characterized in that
%Si + %Mn + %Ni + %Cr > 2.0, or
%Mo > 1.2, or
%B > 2 ppm.

It should be clear that from all the possible compositions within the range only those where the microstructure described in the present invention is attainable are of interest. Some smaller ranges within the above mentioned compositional range are of special significance for certain applications. For example when it comes to the %Ceq content it is preferably to have a minimum value of 0.22%, preferably 0.28%, more preferably 3.2% and even 3.6%. Very high levels of %Ceq are interesting due to the low temperature at which martensite transformation starts, such applications favor %Ceq maximum levels of 0.6%, preferably 0.8% and even 0.9%. %Cr has two ranges of particular interest: 0.6%-1.8% and 2.2%-3.4%. Particular embodiments also prefer %Cr to be 2%. To enhance hardness gradient at the secondary hardness peak it is highly recommendable to have %Moeq present in the steel, often more than 0.4%, preferably more than 1.2%, more preferably more than 1.6% and even more than 2.2% offer a significant effect in this sense. In this particular application of the invention the elements that mostly remain in solid solution, the most representative being %Mn, %Si and %Ni are very critical. It is desirable to have the sum of all elements which primarily remain in solid solution exceed 0.8%, preferably exceed 1.2%), more preferably 1.8% and even 2.6%. As can be seen both %Mn and %Si need to be present. %Mn is often present in an amount exceeding 0.4%, preferably 0.6% and even 1.2%. For particular applications, Mn is interesting to be even 1.5%. The case of %Si is even more critical since when present in significant amounts it strongly contributes to the retarding of cementite coarsening. Therefore %Si will often be present in amounts exceeding 0.4%, preferably exceeding 0.6% and even exceeding0.8%. When the effect on cementite is pursuit then the contents are even bigger, often exceeding 1.2%, preferably 1.5% and even 1.65%. For this purpose A1 can also be used, at least exceeding 0,4%, preferably exceeding 0,5 and even exceeding 0,8%. Also for applications where wear resistance or thermal conductivity are important it is advantageous to use strong carbide formers, then %Zr+%Hf+%Nb+%Ta should be above 0.1%, preferably 1.3% and even 2.2%. Also %V is good carbide former that tends to form quite fine colonies of very hard carbides, thus when wear resistance and toughness are both important, it will generally be used with a content above 0.2%, preferably 0.4% and even more than 0.8%. For very high wear resistance applications it can be used with content higher than 1.2% or even 2.2%. Other elements may be present, especially those with little effect on the objective of the present invention. In general it is expected to have less than 2% of other elements (elements not specifically cited), preferably 1%, more preferably 0.45% and even 0.2%. As can be seen the critical elements for attaining the mechanical properties desired for such applications need to be present and thus it has to be %Si+%Mn+%Ni+%Cr greater than 2.0%, preferably greater than 2.2%, more preferably greater than 2.6% and even greater than 3.2%. For some applications it is interesting to replace %Cr for %Mo, due to the higher effect on the secondary hardness peak and the improved thermal conductivity potential it impairs the steel, and then the same limits apply. Alternatively to %Si+%Mn+%Ni+%Mo > 2.0%.... the presence of %Mo can be dealt alone when present in an amount exceeding 1.2%, preferably exceeding 1.6%, and even exceeding 2.2%. For the applications where cost is important it is specially advantageous to have the expression %Si + %Mn + %Ni + %Cr replaced by %Si + % Mn and then the same preferential limits can apply, but in presence of other alloying elements, also lower limits can be used like %Si+%Mn > 1.1%, preferably 1.4% or even 1.8%. %Ni is desirable to be at least 1%. For this kind of steels tough bainite treatments at temperatures close to martensite start of transformation (Ms) are very interesting (often at least 60%, preferably 70% and more, even more preferably at least 82% of the transformation of austenite should take place below 520 °C, preferably 440 °C, more preferably 410 °C or even 380 °C, but not below 50 °C below martensite start of transformation [Ms]).
The steels described above can be also applied for the manufacturing of big plastic injection tools particularly interesting for applications requiring very low cost steel with high mechanical resistance and toughness. This particular application of the present invention is also interesting for other applications requiring inexpensive steels with high toughness and considerable yield strength. It is particularly advantageous when the steel requires a harder surface for the application and the nitriding or coating step is made coincide with the hardening step.

A contribution to the increase in toughness in the bainitic microstructures of the present invention can be made through the dissolution of the cementite and the carbon that goes into solid solution can contribute to the separation or precipitation of carbides containing carbide-forming elements. Therefore, the present invention is well suited for steels which contain at least 3% carbide formers stronger than iron and thermal treatment is followed by at least one tempering cycle above 500°C to separate the alloy cementite, to dissolve the cementite in solid solution and to separate the carbide formers stronger than iron. (Cr, Mo, W, V, Nb, Zr, Ta, Hf...) often mixed carbides containing those elements and others like for example iron. Those carbides often precipitate as M7C3, M4C3, MC, M6C, M2C and others carbides. The temperature at which this happens is often above 400 °C, preferably 450 °C, more preferably 480 °C and even 540 °C.

For applications where mechanical strength more than wear resistance are important, and it is desirable to attain such mechanical strength without compromising all too much toughness, the volume fraction of small secondary hard particles is of great importance. Small secondary hard particles, in this document, are those with a maximum equivalent diameter (diameter of a circle with equivalent surface as the cross section with maximum surface on the hard particle) below 7.5 nm. It is then desirable to have a volume fraction of small secondary hard particles for such applications above 0.5%. It is believed that a saturation of mechanical properties for hot work applications occurs at around 0.6%, but ithas been observed by the inventors that for some applications requiring high plastic deformation resistance at somewhat lower temperatures it is advantageous to have higher amounts than these 0.6%, often more than 0.8% and even more than 0.94%. Since the morphology (including size) and volume fraction of secondary carbides change with heat treatment, the values presented here describe attainable values with proper heat treatment.

Cobalt has often been used in hot work tool steels principally due to the increase in mechanical strength, and in particular the increase of yield strength maintained up to quite high temperatures. This increase in yield strength is attained trough solid solution and thus it has a quite negative effect in the toughness. The common amounts of Co used for this propose is 3%. Besides the negative effect in toughness it is also well known the negative effect in the thermal conductivity. The inventors have seen that within the compositional ranges of the present invention it is possible to use Co, and attain an improved yield strength/ toughness relation since Co can promote the nucleation of secondary hard particles and thus keep their size small. It has also been seen that for some compositions of the present invention, when adding Co the Thermal diffusivity does indeed decrease at room temperature, but then can actually increase at higher temperatures (normally above 400 °C) if the correct thermo-mechanical treatment is applied. The inventors have seen that the best results are encountered when %Co is above 1.3%, preferably above 1.5% and optimally above 2.4%. Also %C should exceed 3.2%, preferably 3.4% and optimally 3.6%. If thermal conductivity at high temperatures is of outmost importance for the application a special care has to be taken not to have excessive %V, it should be kept below 2.8%, preferably below 2.3% and optimally below 1.7%. Finally %Moeq should normally exceed 3.3% often 3.5% and even 4.0%. Heat treatment has to be selected with a rather high austenitization temperature and an abnormally high tempering temperatures, actually more than 55 HRc commonly achieved with at least one tempering cycle at 630 °C or even above, 50 HRc can be maintained even with one tempering cycle at 660 °C or more. Proper thermo-mechanical processing together with the compositional rules just explained have to be implemented to minimize scattering at high temperatures, the optimized arrangements is characterized by providing diffusivities of more than 5.8 mm2/s, often more than 6.1mm2/s and even more than 6.5mm2/s at measuring temperatures as high as 600 °C.

To increase machinability S, As, Te, Bi or even Pb, Ca, Cu, Se, Sb or others can be used, with a maximum content of 1%, with the exception of Cu, than can even be of 2%. The most common substance, sulfur, has, in comparison, a light negative effect on the matrix thermal conductivity in the normally used levels to increase machinability. However, its presence must be balanced with Mn, in an attempt to have everything in the form of spherical manganese bisulphide, less detrimental for toughness, as well as the least possible amount of the remaining two elements in solid solution in case that thermal conductivity needs to be maximized.

Another hardening mechanism can be used in order to search for some specific combination of mechanical properties or environmental degradation resistance. It is always the intention to maximize the desired property, but trying to have minimal possible adverse impact on thermal conductivity. Solid solution with Cu, Mn, Ni, Co, Si, etc... (including some carbide formers with less affinity to carbon, like Cr) and interstitial solid solution (mainly with C, N and B). For this purpose, precipitation can also be used, with an intermetallic formation like Ni₃Mo, NiAl, Ni₃Ti... (also of Ni and Mo, small quantities of Al and Ti can be added, but special care must be taken for Ti, since it dissolves in M₃Fe₃C carbides and a 2% should be used as a maximum). Finally, other carbide types can also be used, but it is usually difficult to maintain high levels of thermal conductivity, unless carbide formers present a very high affinity with carbon, as it has been described throughout this document. Co can be used as a hardener by solid solution or as a catalyst of Ni intermetallic precipitation, rarely in contents higher than 6%. Some of these elements are also not as harmful when dissolved in M₃Fe₃C carbides, or other carbides of (Fe, Mo, W), this is specially the case for Zr and Hf and, to a lesser extent, for Ta, these can also limit V and Nb solubility.

When amounts are measured in weight percentage, atomic mass and the formed type of carbide determine if the quantity of a used element should be big or small. So, for instance, 2%V is much more than 4%W. V tends to form MC carbides, unless it dissolves in other existing carbides. Thus, to form a carbide unit only a unit of V is needed, and the atomic mass is 50.9415. W tends to form M₃Fe₃C carbides in hot work steels. So three units of W are needed to form a carbide unit, and the atomic mass is 183.85. Therefore, 5.4 more times carbide units can be formed with 2%V than with 4%W.

Tool steel of the present invention can be manufactured with any metallurgical process, among which the most common are sand casting, lost wax casting, continuous casting, melting in electric furnace, vacuum induction melting. Powder metallurgy processes can also be used along with any type of atomization and eventually subsequent compacting as the HIP, CIP, cold or hot pressing, sintering (with or without a liquid phase and regardless of the way the sintering process takes place, whether simultaneously in the whole material, layer by layer or localized), laser cusing, spray forming, thermal spray or heat coating, cold spray to name a few of them. The alloy can be directly obtained with the desired shape or can be improved by other metallurgical processes. Any refining metallurgical process can be applied, like VD, ESR, AOD, VAR... Forging or rolling are frequently used to increase toughness, even three-dimensional forging of blocks. Tool steel of the present invention can be obtained in the form of bar, wire or powder (amongst others to be used as solder or welding alloy). Even, a low-cost alloy steel matrix can be manufactured and applying steel of the present invention in critical parts of the matrix by welding rod or wire made from steel of the present invention. Also laser, plasma or electron beam welding can be conducted using powder or wire made of steel of the present invention. The steel of the present invention could also be used with a thermal spraying technique to apply in parts of the surface of another material. Obviously the steel of the present invention can be used as part of a composite material, for example when embedded as a separate phase, or obtained as one of the phases in a multiphase material. Also when used as a matrix in which other phases or particles are embedded whatever the method of conducting the mixture (for instance, mechanical mixing, attrition, projection with two or more hoppers of different materials...).

Tool steel of the present invention can also be used for the manufacturing of parts under high thermo-mechanical loads and wear resistance or, basically, of any part susceptible to failure due to wear and thermal fatigue, or with requirements for high wear resistance and which takes advantage of its high thermal conductivity. The advantage is a faster heat transport or a reduced working temperature. As an example: components for combustion engines (such as rings of the engine block), reactors (also in the chemical industry), heat exchange devices, generators or, in general, any power processing machine. Dies for forging (open or closed die), extrusion, rolling, casting and metal thixoforming. Dies for plastic forming of thermoplastics and thermosets in all of its forms. In general, any matrix, tool or part can benefit from increased wear resistance and thermal fatigue. Also dies, tools or parts that benefit from better thermal management, as is the case of material forming or cutting dies with release of large amounts of energy (such as stainless steel or TRIP steels) or working at high temperatures (hot cutting, hot forming of sheet).

Additional embodiments are described in the dependent claims.

### EXAMPLES

All values are given in weight percentage.

### Example 1

The following examples show properties that can be obtained:

**Table 1**

| **%C** | **%Mo** | **%W** | **%V** | **%Cr** | **%Si** | **%Mn** | **Other** | **Manteinance T°/time °C / h** | **Hardness / CVN HRc/J** |
|---|---|---|---|---|---|---|---|---|---|
| 0.40 | 0.09 | 0.27 | 0.05 | 2.1 | 1.4 | 1.53 | - | 263 72* | 42 40 |
| 0.39 | 0.05 | 0.2 | 0.02 | <0.01 | 1.5 | 1.6 | Ni, B | 300 72* | 35 34 |
| 0.38 | 0.05 | 0.26 | 0.4 | <0.01 | 1.5 | 1.56 | - | 310 72 | 38 >450** |
| 0.27 | 3.76 | 1.39 | 0.5 | <0.01 | <0.05 | <0.01 | Ni=3.5 Zr, Hf | 230 120* | 41 14 |
| 0.37 | 3.46 | 1.01 | <0.01 | <0.01 | <0.05 | <0.01 | Ni=2.8 | RT slow cool* | 45 >450** |
| 0.33 | 3.8 | 1.22 | 0.4 | 1.06 | 0.1 | <0.01 | Hf, Zr, Nb | 360 72* | 52 250** |
| 0.38 | 3.74 | 1.36 | 0.02 | <0.01 | <0.05 | <0.01 | Zr, Hf, Nb | 280 72* | 50 102** |
| 1.02 | 1.78 | 0.92 | 2.4 | 8.01 | 1.12 | 0.28 | | 250 200* | 60 148** |

| | | | | | | | | | |
|---|---|---|---|---|---|---|---|---|---|
| * Tempering cycles have been applied with at least one tempering in the 520- 680 °C range. **Charpy pendulum resilience was evaluated on a 10x10x55 mm unnotched sample. | | | | | | | | | |

### Example 2

Samples with compositions specified in Table 2 were austenitised at a temperature between 1000-1150°C for about 45 minutes (once the core of the pieces had reached the temperature). Different embodiments of the heat treatment of the present invention where implemented. T_{int,1} was chosen to be in the 500-600 °C range and T_{int,2} was chosen to be in the 320-450 °C range. The rapid cooling to T_{int,1} was made by means of changing the piece to another furnace running at the T_{int,1} temperature and samples were soaked at that temperature for one hour. Afterwards, the temperature further decreased to T_{int,2} in aproximately 2 to 8 hours and afterwards was cooled in air.

**Table2**

| **%C** | **%Mo** | **%W** | **% V** | **%Cr** | **%Si** | **%Mn** | **Other*** | **Hardness after heat treatment HRc** | **Final Hardness / HRc/J** |
|---|---|---|---|---|---|---|---|---|---|
| 0.322 | 3.01 | **1.93** | 0.017 | 0.071 | <0.05 | 0.144 | Ni 3.01 | 40 | 51 / >450 |
| 0.384 | 3.08 | 2.130 | 0.016 | 0.074 | 0.088 | 0.158 | Ni 3.08 | 338HB | 48/416 |
| 0.384 | 3.09 | 2.08 | 0.019 | 0.079 | 0.104 | 0.168 | Ni 3.11 | 348HB | 48/>450 |
| 0,31 | 3,70 | 2,3 | <0.005 | 0,01 | 0,02 | 0,02 | Ni 1,86 | 41 | 50 |
| 0,37 | 3,90 | 2,0 | <0.005 | 0,01 | 0,02 | 0,11 | Ni 2,05 | 40 | 48 |
| 0,39 | 3,71 | 1,2 | 0,6 | 0,01 | 0,05 | 0,02 | Ni 0,84, Hf, Nb,Zr | 42 | 53.5 |
| 0.39 | 3.57 | 1.35 | 0.44 | <0.01 | <0.01 | <0.01 | Hf, Zr, Nb | 47 | 52 |
| 0,21 | 3,2 | 1,04 | 0,3 | 0,01 | 0,04 | 0,21 | - | 45 | 48 |
| 0,294 | 3,290 | 1,440 | <0.01 | 0,053 | 0,213 | 0,111 | - | 40 | 49 |

| | | | | | | | | | |
|---|---|---|---|---|---|---|---|---|---|
| *Elements specified as other are present, otherwise indicated, in an amount of less than 2% | | | | | | | | | |

### Example 3

Samples with compositions specified in Table 1 were austenitised at a temperature between 1000-1100°C for about 45 minutes (once the core of the pieces had reached the temperature). Different embodiments of the heat treatment of the present invention where implemented. T_{int,1} was chosen to be in the 500-600 °C range and T_{int,2} was chosen to be in the 320-450 °C range. The rapid cooling to T_{int,1} was made in two steps: a first step comprising rapid cooling to the range 500-600 °C, a second step of heating to a temperature within the same temperature range but higher and cooling again to the first temperature within the same range 500-600 °C by means of changing the piece to another furnace running at the T_{int,1} temperature and samples were soaked at that temperature for one hour. Afterwards, the temperature further decreased to T_{int,2} in aproximately 3 to 10 hours and afterwards was cooled in air.

**Table 3**

| **%C** | **%Mo** | **%W** | **%V** | **%Cr** | **%Si** | **%Mn** | **Other *** | **Hardness after heat treatment HRc** | **Final Hardness / HRc / J** |
|---|---|---|---|---|---|---|---|---|---|
| 0.322 | 3.01 | 1.93 | 0.017 | 0.071 | <0.05 | 0.144 | Ni 3.01 | 44 | 52 / 326 |
| 0.384 | 3.08 | 2.13 0 | 0.016 | 0.074 | 0.088 | 0.158 | Ni 3.08 | 385HB | 48/260 |
| 0.384 | 3.09 | 2.08 | 0.019 | 0.079 | 0.104 | 0.168 | Ni 3.11 | 382HB | 48/435 |
| 0,31 | 3,70 | 2,3 | <0.0 05 | 0,01 | 0,02 | 0,02 | Ni 1,86 | 41 | 49 |
| 0,37 | 3,90 | 2,0 | <0.0 05 | 0,01 | 0,02 | 0,11 | Ni 2,05 | 41 | 48.5 |

| | | | | | | | | | |
|---|---|---|---|---|---|---|---|---|---|
| *Elements specified as other are present, otherwise indicated, in an amount of less than 2% | | | | | | | | | |

## Claims

1. A method to manufacture a steel, casting die or tool, wherein the steel has the following composition, all percentages being indicated in weight percent:
| | | | | | | | |
|---|---|---|---|---|---|---|---|
| %C_{eq} | = 0.16 - 1.9 | %C | = 0.16 - 1.9 | %N | = 0 - 1.0 | %B | =0 - 0.6 |
| %Cr | < 1.8 | %Ni | =0 - 6 | %Si | = 0 - 1.4 | %Mn | = 0 - 3 |
| %Al | =0 - 2.5 | %Mo | =0 - 10 | %W | =0-10 | %Ti | =0-2 |
| %Ta | = 0 - 3 | %Zr | = 0 - 3 | %Hf | = 0 - 3 | %V | = 0 - 4 |
| %Nb | = 0 - 1.5 | %Cu | = 0 - 2 | %Co | = 0 - 6 | | |
the rest consisting of iron and trace elements wherein, $% {C}_{eq} = % ⁢ C + 0.86 ∗ % ⁢ N + 1.2 ∗ % ⁢ B ,$ and
%Mo + ½ · %W > 2.0,
comprising providing a steel with both a bainite and a martensite domain of existence, wherein the steel is subjected to a thermal treatment comprising the following steps:
a) Austenitization,
b) Cooling while avoiding the formation of more than a 20% stable phases with a transformation temperature higher than bainite,
c) Maintaining the temperature to transform at least 60% vol of remaining austenite between Ms+300°C and Ms-50°C, wherein Ms is the martensite start of transformation temperature;
wherein more than 80% of the microstructure is bainitic with fine carbide-like constituents with a CVN higher than 8 Joule within at least 20mm from the surface of the thermally treated steel.

2. The method according to claim 1, wherein the steel has a martensite start (Ms) of transformation equal or lower than 480°C

3. The method according to any of claims 1 or 2, wherein the steel contains at least 3% carbide formers stronger than iron and the thermal treatment is followed by at least one tempering cycle above 500°C to separate the alloy cementite, to dissolve the cementite in solid solution, and to separate the carbide formers stronger than iron.

4. The method according to any of claims 1 to 3, wherein the steel contains at least 0.4% Si and/or 0.4% A1 to retard the cementite growth.

5. The method according to any of claims 1 or 4 wherein, upon formation of the bainite, the steel is tempered with at least one tempering cycle at a temperature above 500°C to ensure that a portion of the cementite is replaced by carbide-like structures containing carbide formers stronger than iron.

6. The method according to any of claims 1 to 5, wherein the steel is a high thermal conductivity steel and that at the least one tempering cycle is carried out at a temperature above 540°C, providing a low scattering structure **characterized by** a thermal diffusivity higher than 8 mm²/s.

7. The method according to any of claims 1 to 6, wherein at least 70% of the bainitic transformation is made at temperature below 400°C, attaining a microstructure of fine bainite **characterized by** a hardness above 45 HRc without tempering.

8. The method according to any of claims 1 to 7, wherein at least 70% of the bainitic transformation is made at temperatures below 400°C and/or the thermal treatment includes at least one tempering cycle at a temperature above 500°C to ensure separation of stronger carbide formers carbides, so that most of the attained microstructure, with the exception of the eventual presence of primary carbides, is **characterized by** the minimization of rough secondary carbides, in particular at least 60% in volume of the secondary carbides has a size of 250 nm or less, such that a toughness of 10 J CVN or more is attained.

9. The method according to any of claims 1 to 8, wherein the composition and tempering strategy is chosen so that high temperature separation secondary carbide types such as types MC, MC-like type as M4C3, M6C and M2C are formed, in such a manner that a hardness above 47 HRc is obtainable even after holding the material for 2h at a temperature of 600 °C.

10. The method according to any of claims 1 to 9, wherein the steel has a composition within the following range:
% Cr < 3.0
% Si < 0.8
wherein
%Mo + ½ · %W > 2.0.
and the tempering strategy is chosen to minimize carriers scattering, such that a low scattering structure **characterized by** a diffusivity of 8 mm²/s or more is obtainable even for a hardness of 45 HRc or more.

11. The method according to any of claims 1 to 9, wherein the steel has the following composition:
% Ni > 0.8

12. The method according to any of claims 1 to 11, **characterized in that** the steel presents at least two of the following features:
- it contains retained austenite;
- its cementite is not wholly dissolved in the solid solution;
- its cementite has not fully coalesced; and
- carbide formers stronger than iron are present in the solid solution,
so that the hardness of the steel can be raised in an amount of at least 4 HRc upon application of a later thermal treatment below austenitizing temperature.

## Patentansprüche

1. Verfahren zur Herstellung eines Stahls, einer Gießform oder eines Werkzeugs, wobei der Stahl die folgende Zusammensetzung aufweist, wobei alle Prozentangaben in Gewichtsprozent angegeben sind:
| | | | |
|---|---|---|---|
| %C_{eq} = 0,16 - 1,9 | % C = 0,16 - 1,9 | %N = 0 - 1,0 | %B = 0 - 0,6 |
| %Cr < 1,8 | %Ni = 0 - 6 | %Si = 0 - 1,4 | %Mn = 0 - 3 |
| %Al = 0 - 2,5 | %Mo = 0 - 10 | %W = 0 - 10 | %Ti =0-2 |
| %Ta = 0 - 3 | %Zr = 0 - 3 | %Hf =0-3 | %V =0-4 |
| %Nb = 0 - 1,5 | %Cu =0-2 | %Co = 0 - 6 | |
der Rest bestehend aus Eisen und Spurenelementen, wobei, $% {C}_{eq} = % ⁢ C + 0,86 ∗ % ⁢ N + 1,2 ∗ % ⁢ B ,$ und
%Mo + ½ · %W > 2,0,
das die Erziehlung eines Stahls mit sowohl einer Bainit- als auch einer Martensit-Existenzdomäne umfasst, wobei der Stahl einer Wärmebehandlung unterzogen wird, die die folgenden Schritte umfasst:
a) Austenitisierung,
b) Abkühlen unter Vermeidung der Bildung von mehr als 20% stabilen Phasen mit einer Transformationstemperatur höher als Bainit,
c) Aufrechterhalten der Temperatur zur Umwandlung von mindestens 60% vol verbleibendem Austenit zwischen Ms+300°C und Ms-50°C, wobei Ms die Starttemperatur der Martensit-Umwandlung ist;
wobei mehr als 80% der Mikrostruktur bainitisch ist mit feinen karbidartigen Konstituenten mit einem CVN höher als 8 Joule innerhalb von mindestens 20 mm von der Oberfläche des wärmebehandelten Stahls.

2. Verfahren nach Anspruch 1, wobei der Stahl einen Martensit-Umwandlungsstart (Ms) von 480°C oder niedriger aufweist.

3. Verfahren nach einem der Ansprüche 1 oder 2, wobei der Stahl mindestens 3% Karbidbildner enthält, die stärker als Eisen sind, und auf die Wärmebehandlung mindestens ein Anlasszyklus über 500°C folgt, um den Zementit zu trennen und den Zementit in fester Lösung zu lösen, und Karbidbildner stärker als Eisen aus der festen Lösung herauszubringen.

4. Verfahren nach einem der Ansprüche 1 bis 3, wobei der Stahl mindestens 0,4% Si und / oder 0,4% Al enthält, um das Zementitwachstum zu verzögern.

5. Verfahren nach einem der Ansprüche 1 oder 4, wobei der Stahl nach Bildung des Bainits mit mindestens einem Temperzyklus bei einer Temperatur über 500°C getempert wird, um sicherzustellen, dass ein Teil des Zementits durch karbidähnliche Strukturen ersetzt wird, die Karbidbildner stärker als Eisen enthalten.

6. Verfahren nach einem der Ansprüche 1 bis 5, wobei der Stahl ein Stahl mit hoher Wärmeleitfähigkeit ist und an dem mindestens ein Temperzyklus bei einer Temperatur über 540°C durchgeführt wird, wobei eine Struktur mit geringer Streuung erzeugt wird, die durch eine thermische Diffusivität von höher als 8 mm²/ s gekennzeichnet ist.

7. Verfahren nach einem der Ansprüche 1 bis 6, wobei mindestens 70% der bainitischen Umwandlung bei einer Temperatur unter 400°C durchgeführt wird, wodurch eine Mikrostruktur aus feinem Bainit erhalten wird, die durch eine Härte über 45 HRc ohne Tempern gekennzeichnet ist.

8. Verfahren nach einem der Ansprüche 1 bis 7, wobei mindestens 70% der bainitischen Umwandlung bei Temperaturen unter 400°C durchgeführt werden und / oder die Wärmebehandlung mindestens einen Temperzyklus bei einer Temperatur über 500°C umfasst, um die Abtrennung von stärkeren Karbidbildnern Karbiden sicherzustellen, so dass der größte Teil der erzielten Mikrostruktur, mit Ausnahme des eventuellen Vorhandenseins von Primärkarbiden, durch die Minimierung von groben Sekundärkarbiden gekennzeichnet ist, insbesondere mindestens 60 % des Volumen der Sekundärkarbide eine Größe von 250 nm oder weniger hat, so dass eine Zähigkeit von 10 J CVN oder mehr erreicht wird.

9. Verfahren nach einem der Ansprüche 1 bis 8, wobei die Zusammensetzung und die Temperstrategie so gewählt werden, dass Hochtemperaturtrennungs-sekundär-Karbidtypen, wie die Typen MC, MC-artige Typen wie M4C3, M6C und M2C, auf solche Weise gebildet werden, dass eine Härte über 47 HRc erzielbar ist, sogar auch nach 2-stündigem Halten des Materials bei einer Temperatur von 600 °C.

10. Verfahren nach einem der Ansprüche 1 bis 9, wobei der Stahl eine Zusammensetzung im folgenden Bereich aufweist:
% Cr < 3,0
% Si < 0,8
wobei
% Mo + ½ · %W > 2,0.
und die Temperstrategie so gewählt wird, dass die Trägerstreuung minimiert wird, so dass eine Struktur mit geringer Streuung, die durch ein Diffusivität von 8 mm²/s oder mehr gekennzeichnet ist, erzielt werden kann, selbst für eine Härte von 45 HRc oder höher.

11. Verfahren nach einem der Ansprüche 1 bis 9, wobei der Stahl die folgende Zusammensetzung aufweist:
% Ni > 0,8

12. Verfahren nach einem der Ansprüche 1 bis 11, **dadurch gekennzeichnet, dass** der Stahl mindestens zwei der folgenden Merkmale aufweist:
- er enthält Restaustenit;
- sein Zementit ist nicht vollständig in der festen Lösung gelöst;
- sein Zementit ist nicht vollständig koalesziert; und
- die feste Lösung enthält Karbidbildner, die stärker als Eisen sind,
so dass die Härte des Stahls bei Anwendung einer späteren Wärmebehandlung unterhalb der Austenitisierungstemperatur um einen Betrag von mindestens 4 HRc erhöht werden kann.

## Revendications

1. Un procédé pour fabriquer un acier, modèle de fonderie ou outil, dans lequel l'acier a la composition suivante, tous les pourcentages étant indiqués en pourcentages en poids :
| | | | | | | | |
|---|---|---|---|---|---|---|---|
| %C_{eq} | = 0,16 - 1,9 | %C | = 0,16 - 1,9 | %N | = 0 - 1,0 | %B | = 0 - 0,6 |
| %Cr | < 1,8 | %Ni | = 0 - 6 | %Si | = 0 - 1,4 | %Mn | = 0 - 3 |
| %A1 | = 0 - 2,5 | %Mo | =0 - 10 | %W | = 0 - 10 | %Ti | = 0 - 2 |
| %Ta | = 0 - 3 | %Zr | = 0 - 3 | %Hf | = 0 - 3 | %V | = 0 - 4 |
| %Nb | = 0 - 1,5 | %Cu | = 0 - 2 | %Co | = 0 - 6 | | |
le reste comprenant du fer et des éléments à l'état de trace, dans lequel, $% {C}_{eq} = % ⁢ C + 0,86 ∗ % ⁢ N + 1,2 ∗ % ⁢ B ,$ et
%Mo + ½ · %W > 2,0,
comprenant la fourniture d'un acier ayant à la fois un domaine d'existence de bainite et de martensite, dans lequel l'acier est soumis à un traitement thermique comportant les étapes suivantes :
a) Austénitisation,
b) Refroidissement tout en évitant la formation de plus de 20% de phases stables avec une température de transformation supérieure à la bainite,
c) Maintien de la température pour transformer au moins 60% en volume de l'austénite restante entre Ms+300°C et Ms-50°C, où Ms est le démarrage de martensite de la température de transformation ;
dans lequel plus de 80% de la microstructure est bainitique avec de fins constituants à l'apparence de carbures avec un CVN supérieur à 8 Joule dans au moins 20 mm à partir de la surface de l'acier traité thermiquement.

2. Le procédé selon la revendication 1, dans lequel l'acier a un démarrage de martensite (Ms) de transformation égal ou inférieur à 480°C.

3. Le procédé selon l'une des revendications 1 ou 2, dans lequel l'acier contient au moins 3% de matières carbures plus résistantes que le fer et le traitement thermique est suivi par au moins un cycle de revenu supérieur à 500°C pour séparer the la cémentite d'alliage, pour dissoudre la cémentite en solution solide, et pour séparer les matières carbures plus résistantes que le fer.

4. Le procédé selon l'une des revendications 1 à 3, dans lequel l'acier contient au moins 0,4% Si et/ou 0,4% Al pour retarder la croissance de la cémentite.

5. Le procédé selon l'une des revendications 1 ou 4 dans lequel, dès la formation de la bainite, l'acier est trempé avec au moins un cycle de revenu à une température supérieure à 500°C pour s'assurer qu'une partie de la cémentite est remplacée par des structures à l'apparence de carbures contenant des matières carbures plus résistantes que le fer.

6. Le procédé selon l'une des revendications 1 à 5, dans lequel l'acier est un acier à haute conductivité thermique et dans lequel le au moins un cycle de revenu est réalisé à une température supérieure à 540°C, ce qui fournit une structure à basse diffusion **caractérisée par** une diffusivité thermique supérieure à 8 mm²/s.

7. Le procédé selon l'une des revendications 1 à 6, dans lequel au moins 70% de la transformation bainitique est faite à une température inférieure à 400°C, permettant d'obtenir une microstructure de fine bainite **caractérisée par** une dureté supérieure à 45 HRc sans revenu.

8. Le procédé selon l'une des revendications 1 à 7, dans lequel au moins 70% de la transformation bainitique est faite à des températures inférieures à 400°C et/ou le traitement thermique comprend au moins un cycle de revenu à une température supérieure à 500°C pour garantir la séparation des carbures de matières carbures plus fortes, de façon que la plus grande partie de la microstructure obtenue, à l'exception de la présence éventuelle de carbures primaires, soit **caractérisée par** la minimisation des carbures secondaires irréguliers, en particulier au moins 60% en volume des carbures secondaires a une taille de 250 nm ou moins, de sorte qu'une dureté de 10 J CVN ou plus est obtenue.

9. Le procédé selon l'une des revendications 1 à 8, dans lequel la composition et la stratégie de revenu sont choisies pour que lors de la séparation à haute température des types de carbures secondaires tels que les types MC, le type similaire à MC comme M4C3, M6C et M2C soient formés, de telle façon qu'une dureté supérieure à 47 HRc puisse être obtenue même après avoir maintenu le matériau pendant 2 h à une température de 600°C.

10. Le procédé selon l'une des revendications 1 à 9, dans lequel l'acier a une composition comprise dans la gamme suivante :
% Cr < 3,0
% Si < 0,8
dans lequel
%Mo + ½ · %W > 2,0.
et la stratégie de revenu est choisie pour minimiser la diffusion de porteurs, pour qu'une structure à basse diffusion **caractérisée par** une diffusivité de 8 mm²/s ou plus puisse être obtenue même pour une dureté de 45 HRc ou plus.

11. Le procédé selon l'une des revendications 1 à 9, dans lequel l'acier a la composition suivante :
% Ni > 0,8

12. Le procédé selon l'une des revendications 1 à 11, **caractérisé en ce que** l'acier présente au moins deux des caractéristiques suivantes :
- il contient de l'austénite retenue ;
- sa cémentite n'est pas complètement dissoute dans la solution solide ;
- sa cémentite n'a pas totalement coalescé ; et
- des matières carbures plus fortes que le fer sont présentes dans la solution solide,
pour que la dureté de l'acier puisse être élevée dans une proportion d'au moins 4 HRc dès l'application d'un dernier traitement thermique en dessous de la température d'austénitisation.
